

## UNITED STATES PATENT OFFICE

SHINJIRO HORII, OF TOKYO, JAPAN

## STENCIL SHEET

No Drawing.

Application filed June 20, 1928. Serial No. 287,051.

My invention relates to improvements in stencil sheets of the type commonly used for autographic and typewriting duplication, consisting of a sheet of fibrous material having a coating which is impermeable to ink and can be stencilized by the pressure of a writing stylus or by the impact of the type of a writing machine.

It has previously been proposed to produce 10 a stencil sheet of this kind such as a base of fibrous material, having Japanese Yoshino paper, coated with a composition including a cellulose ester, such as cellulose acetate or nitrate, dissolved in a volatile solvent, such as alcohol-ether mixture or amyl acetate, and a tempering agent such as castor oil, soya bean oil, hydro-carbon oil or oleic acid.

It has also been proposed to produce such 20 a stencil sheet having a fibrous base which is coated with a composition including esters of polysaccharides and a tempering agent such as naphthenic acid glycerides, chlorinated naphthalene or fatty acid of tsubaki oil.

25 The stencil sheet of the present invention comprises a fibrous base coated with a coating material consisting of a solution of esters of polysaccharides in a volatile solvent in admixture with dolphin oil.

30 Dolphin oil is obtained from the blubber of the various species of dolphin belonging to the Delphinidae, such as, *Delphinus longirostris*, Gray (mairuka), *Delphinus globiceps*, Lam. (black fish or bottlenose dolphin), *Lagenorhynchus acutus*, Gray (kamairuka), *Delphinus phocana*, L. (brown porpoise), *Phocoena communis*, Less. (nezumi iruka), *Globiocephalus sieboldii*, Gray (pilot-whale) etc.

40 The oils from the jaw and from the body differ considerably in composition. These oils contain notable amounts of sperm-aceti, forming intermediate members between fatty oils and liquid waxes. Moreover, these oils 45 occupy an exceptional position on account of their containing considerable proportions of glycerides of volatile acids.

In this connection it may be noted that the 50 employment of a marine wax, such as spermaceti, sperm oil, bottle-nose oil, or other

analogous substances derived from the allied species of salt-water fish in admixture with fatty oils, fats or fatty acids has been proposed in the production of stencil sheets. It has also been suggested to produce a stencil 55 sheet of a fibrous base having a type impres- sheet of a fibrous base having a type impres- sible coating thereon, consisting of a base of lac dissolved in alcohol, and having added thereto dissolved nitrated cotton, camphor, castor oil and sperm oil. Spermaceti or sperm 60 oil is a true wax, in solid or fluid state, consisting chiefly of compound esters of fatty acids and monovalent alcohols. It is found, however, that sperm oil in association with esters of polysaccharides as a tempering 65 agent, is entirely unsuitable, having the draw- back of being a coating not sufficiently tough and being easily crumbled or cracked on the surface when handled. According to the 70 present invention, the ink-proof coating consists of a homogeneous mixture of esters of polysaccharides and dolphin oil. Dolphin oil forms an intermediate link between whale oil (consisting nearly wholly of glycerides) and sperm oil (a true wax). Dolphin oil has 75 a suitable density and limpidity even at low temperatures, and, when it is used in the production of a stencil sheet for coating the same, in admixture with the esters of polysaccharides, the coating is perfect and uniform, and 80 a stencil sheet is produced which is easily stencilized making clear impressions.

In the practice of the invention, a sheet of fibrous base, such as Japanese Yoshino paper, is coated or impregnated with a coating ma- 85 terial prepared by esters of polysaccharides, such as starch acetate, mannan acetate, cel- lulose acetate and cellulose nitrate, being dis- solved in a suitable solvent, such as acetone, 90 alcohol, ethyl acetate, amyl acetate, benzine and benzol, or a mixture of them, to which dolphin oil has been added.

To a given quantity of this material a suit- 95 able quantity of whale oil, neat's foot oil, lard oil or naphthenic acid glycerides may be added in admixture with the dolphin oil. And also, if desired, a tempering agent such as hydrocarbon oils, fatty oils, naphthenic acid glycerides, oils, fats, fatty acids, waxes, triacetin, butyl tartrate, ethyl or butyl phtha- 100

late, triphenyl or tricresyl phosphate, or a mixture of them may be added to the above described coating material. The coating material may be added into the paper stuff in a mixing hollander during the paper making operation.

The proportions of the ingredients of the composition may vary according to several circumstances. The following is an example:

|                            | Parts by weight |
|----------------------------|-----------------|
| 10 Cellulose nitrate       | 10              |
| Amyl acetate               | 20              |
| Ethyl acetate              | 30              |
| Ethyl alcohol              | 20              |
| 15 Benzol                  | 30              |
| Dolphin oil                | 25              |
| Naphthenic acid glycerides | 5               |

The term "esters of polysaccharides" is intended to include not only one of definite esters of polysaccharides, but also a mixture of them.

What I claim is:

1. A stencil sheet adapted for stencilizing by pressure, consisting of a base of fibrous material having a coating including esters of polysaccharides and dolphin oil.
2. A stencil sheet adapted for stencilizing by pressure, consisting of a base of fibrous material having a coating including esters of polysaccharides, dolphin oil, and tempering agents.
3. A stencil sheet adapted for stencilizing by pressure, consisting of a base of fibrous material having a coating including esters of polysaccharides, dolphin oil, and other oils.

In testimony whereof I affix my signature.

SHINJIRO HORII.

40

45

50

55

60

65